

Sept. 15, 1964

F. A. MLAGARI, JR

3,148,979

AUSTENITIC STEEL

Filed Oct. 31, 1962

5 Sheets-Sheet 1

FIG.2



FIG.1



Sept. 15, 1964

F. A. MLAGARI, JR

3,148,979

AUSTENITIC STEEL

Filed Oct. 31, 1962

5 Sheets-Sheet 2

FIG.4



FIG.3



Sept. 15, 1964

F. A. MALAGARI, JR

3,148,979

AUSTENITIC STEEL

Filed Oct. 31, 1962

5 Sheets-Sheet 3

FIG.5



Sept. 15, 1964

F. A. MALAGARI, JR

3,148,979

AUSTENITIC STEEL

Filed Oct. 31, 1962

5 Sheets-Sheet 4



Sept. 15, 1964

F. A. MALAGARI, JR

3,148,979

AUSTENITIC STEEL

Filed Oct. 31, 1962

5 Sheets-Sheet 5



1

3,148,979  
AUSTENITIC STEEL

Frank A. Malagari, Jr., Freeport, Pa., assignor to Allegheny Ludlum Steel Corporation, Brackenridge, Pa., a corporation of Pennsylvania

Filed Oct. 31, 1962, Ser. No. 234,439  
11 Claims. (Cl. 75—124)

This invention relates to a new composition of matter and relates in particular to a new austenitic steel which exhibits high strength and oxidation resistance properties.

Austenitic steels of the aluminum-manganese variety have recently been developed which possess strength properties far in excess of those possessed by the conventional chromium-nickel stainless steels. Such compositions develop higher strength by age hardening than the commercially available austenitic age hardening grades, and annealed tensile properties are also much higher than for such known austenitic stainless steels. The aluminum-manganese austenitic steels were originally intended to be inexpensive stainless steels in that the relatively inexpensive and non-critical elements aluminum and manganese were substituted for the conventional chromium and nickel. Although such compositions have relatively poor corrosion and oxidation resistance properties, these steels, the most common of which contains from about 7% to 16% aluminum, 20% to 40% manganese, 0.01% to 1.1% carbon and the balance iron, have proved to have mechanical properties that far exceed those of the conventional austenitic stainless steels at both room and elevated temperatures. For example, certain of the aluminum-manganese steels have been found to have yield strengths of up to about 70,000 p.s.i. at room temperature and up to about 69,000 p.s.i. at 649° C. (1200° F.) as compared to about 35,000 p.s.i. and 12,000 p.s.i. respectively for AISI Type 304 stainless steel. Being austenitic, such aluminum-manganese steels work harden and, since they contain substantial quantities of aluminum, possess a low density. Hence, these steels not only possess superior strength properties to stainless steel, but also are lighter.

Although the oxidation resistance of the aluminum-manganese steels at relatively elevated temperatures has been alleged to be good, such properties have been found to be inferior to stainless steel at temperatures exceeding about 871° C. (1600° F.). Such lack of oxidation resistance has markedly detracted from the advantageous properties of the aluminum-manganese steels since most applications of steel requiring high strength properties, particularly at elevated temperatures, also require good oxidation resistance.

It has now been found that the oxidation resistance of certain of the aluminum-manganese steels may be significantly increased by additions of critical amounts of both chromium and nickel. Hence, the present invention is directed to a low density, oxidation resistant, ductile austenitic steel having aluminum, manganese, chromium, nickel and carbon present within specified critical ranges. The present compositions are not only ductile and formable, but have strength properties exceeding those of comparative stainless steels and oxidation resistance properties exceeding those of the known aluminum-manganese compositions and the austenitic stainless steels.

Additionally, it has been discovered that the steel of the present invention possesses electrical resistivity properties which, when coupled with its oxidation resistance, renders it an ideal electrical heating element material. Such steel has been found to possess significantly improved properties over the more expensive nickel-base alloys being employed for such applications. The present steel has also been found to possess a coefficient of resistance change vs. temperature property that is far superior to

2

similar properties of the conventional heater materials. Still further, since the present steel possesses a substantially austenitic structure, it suffers no magnetostriction change in physical dimensions due to the influence of alternating current, and consequently is an ideal material for use as heating elements or other electrical applications where noise is a factor.

Such discoveries are significant since the aluminum-manganese-chromium-nickel-carbon steel of the present invention is ductile and may be readily formed into wire, and the electrical resistivity is significantly higher than the well known 80% nickel-20% chromium alloy, referred to hereinafter as Alloy A, and which is now commonly employed for such applications as electrical heater units. The oxidation resistance properties of the composition of the present invention are equivalent to or exceed those of Alloy A. Further, the present composition is less expensive than Alloy A which contains about 80% nickel and 20% chromium, both of which are relatively expensive and critical elements.

It is, accordingly, an object of the present invention to provide a ductile, oxidation resistant, high strength, low density steel.

It is also an object of the present invention to provide a ductile and formable austenitic steel which possesses higher strength properties than stainless steel and excellent oxidation resistance properties.

A further object of the present invention is to provide a formable steel that may be fabricated into wire that has good electrical resistance and oxidation resistance properties that render it suitable for use as electrical resistance heating elements.

A still further object of the present invention is to provide a material having an excellent coefficient of resistance change vs. temperature properties.

Still another object of the present invention is to provide an austenitic steel having the property of being free from noise-emitting magnetostriction changes in physical dimensions when subjected to alternating electric currents.

Other objects and advantageous features will be obvious from the following description and the accompanying drawings wherein:

FIGURE 1 is a graph showing the rate of oxidation of a steel of the present invention as compared with a known iron-carbon-manganese-aluminum steel at temperatures ranging from 760° C. (1400° F.) to 1149° C. (2100° F.);

FIG. 2 is a graph showing the effect of varying the chromium contents of the steel of the present invention on oxidation resistance and illustrates the necessity for and criticality of the chromium range;

FIG. 3 is a graph showing the effect of varying the nickel contents of the steel of the present invention on oxidation resistance and illustrates the necessity for and criticality of the nickel range;

FIG. 4 is a graph showing the effect of varying the aluminum content of the steel of the present invention on oxidation resistance and illustrates the necessity for and criticality of the aluminum range;

FIG. 5 is a graph showing the combined effects of nickel, chromium and aluminum and the effect of such elements within their critical range limitations, on the oxidation resistance of the present compositions;

FIG. 6 is a lower left hand portion of a triaxial diagram showing the oxidation resistance properties of steels containing four different aluminum contents and having varying nickel and chromium contents; and

FIG. 7 is a graph the curves of which represent the coefficient of resistance vs. temperature for a steel of the present invention and for the Alloy A identified hereinbefore.

In general this invention relates to a new steel having an analysis in the range of 0.50% to 1.0% carbon, 17% to 30% manganese, 8% to 12% aluminum, 1.0% to 12% nickel, 3% to 11% chromium and the balance iron with incidental impurities. Preferably, in order to obtain optimum oxidation resistance, the analysis is within the range of 0.75% to 1.0% carbon, 17% to 30% manganese, 9% to 12% aluminum, 3% to 8% nickel, 5% to 10% chromium, and the balance iron with not more than 0.5% of incidental impurities.

In the steels of this invention carbon and manganese are required in the ranges given in order to stabilize the austenitic structure of the steel. Thus if the steel contains less than 0.5% carbon, the steel may contain undesirable quantities of unstable austenite and transformation products thereof. Preferably the carbon should be maintained at not less than 0.75% although not in excess of about 1.0% as greater amounts may have an adverse effect on workability and the corrosion resistance properties. Likewise, the manganese should be maintained at not less than about 17% so as to maintain a stable austenitic structure but should not exceed about 30% as greater amounts thereof will have an adverse effect on the strength properties of the resulting steel.

The steels of this invention are characterized by high oxidation resistance, good strength and ductility, low density, high electrical resistivity, low coefficient of resistance change vs. temperature, and are free of magnetostriction change in dimensions when subjected to alternating electrical currents.

As stated hereinbefore the present steel is an improvement over the known aluminum-manganese-carbon-iron steels. A representative steel of the prior known system is one (Heat No. 9X686) having an analysis of 0.92% carbon, 24.25% manganese, 0.013% phosphorus, 0.005% sulfur, 0.16% silicon, 9.8% aluminum, 0.20% chromium and the balance iron. In order to show the improvement of the present steel in oxidation resistance, reference is made to a steel (Heat No. GB-94) having an analysis of 1.02% carbon, 24.54% manganese, 0.014% phosphorus, 0.009% sulfur, 0.038% silicon, 9.72% aluminum, 3.56% nickel, 5.01% chromium and the balance iron. Such steels were subjected to different test temperatures in air for times of from 60 to 100 hours and the weight gain of the oxidation was measured. Referring to FIG. 1, the results of such oxidation tests are graphically illustrated by curves 10 and 12 representing the weight gain in mg./cm.<sup>2</sup> on the steels at the different test temperatures with curve 10 being based on Heat No. 9X686 and curve 12 being based on Heat No. GB-94. As clearly illustrated, the controlled addition of chromium and nickel greatly improves and imparts outstanding oxidation resistance to the steel.

In order to more clearly illustrate the effect of chromium on the steel of this invention, reference may be had to the following Table I in which are listed a number of steels having chromium contents ranging from 0% to 10% for a composition in which carbon is 0.78% to 1.03%, manganese is 16.9% to 27%, aluminum is 8.74% to 9.8% and nickel is 2.8% to 3.85% and the results of oxidation tests thereon at 1093° C. (2000° F.) for times in excess of 50 hours with the exception of FR-34 which was tested only 1 hour.

Table I

| Heat No. | C    | Mn    | P    | S    | Si   | Al   | Ni   | Cr   | Weight Gain, Mg/cm. <sup>2</sup> |
|----------|------|-------|------|------|------|------|------|------|----------------------------------|
| FR-34    | .97  | 23.97 | .013 | 0.15 | .180 | 9.32 | 3.85 | —    | 10.10                            |
| GI-40    | 1.01 | 16.93 | .020 | .009 | .070 | 9.46 | 2.92 | 4.90 | 0.0                              |
| GI-38    | 1.02 | 19.58 | .030 | .009 | .100 | 9.00 | 2.88 | 5.01 | 1.03                             |
| GB-94    | 1.02 | 24.54 | .014 | .009 | .088 | 9.72 | 3.56 | 5.01 | 0.50                             |
| GI-42    | .78  | 25.69 | .014 | .014 | .085 | 9.73 | 3.46 | 5.13 | 0.16                             |
| GI-44    | 1.03 | 26.15 | .017 | .014 | .047 | 9.80 | 3.42 | 7.25 | 1.10                             |
| GI-45    | 1.03 | 26.18 | .018 | .017 | .100 | 9.26 | 3.43 | 9.34 | 0.91                             |
| RV-760   | .99  | 24.60 | .006 | .009 | .045 | 8.74 | 3.49 | 9.99 | 0.21                             |

Referring to FIG. 2, curve 14 is a graphic illustration of the oxidation tests on the steels of Table I and clearly illustrates that the chromium content should be maintained in excess of 3% and preferably in the range of 5% to 10% for best results. Above 10% chromium appears to have a detrimental effect on the ductility of the resulting steel.

The effect of nickel is illustrated by reference to the steels of the following Table II and in which the nickel varies from 0.15% to 12% where the other elements are in the range of 0.78% to 1.02% carbon, 8.6% to 9.75% aluminum, 16.93% to 27.36% manganese and from 4.9% to 5.36% chromium and in which the oxidation results as tested at 1093° C. (2000° F.) for times in excess of 50 hours are listed.

Table II

| Heat No. | C    | Mn    | P    | S    | Si   | Al   | Ni    | Cr   | Weight Gain, mg./cm. <sup>2</sup> |
|----------|------|-------|------|------|------|------|-------|------|-----------------------------------|
| GI-47    | 1.01 | 27.36 | .018 | .012 | .066 | 9.19 | 0.15  | 5.36 | 86.2                              |
| RV-650   | .99  | 20.16 | .003 | .011 | .066 | 8.60 | 0.50  | 5.00 | 13.0                              |
| RV-649   | .99  | 19.93 | .008 | .012 | .070 | 9.08 | 2.07  | 5.04 | 6.6                               |
| GI-38    | 1.02 | 19.58 | .030 | .009 | .100 | 9.00 | 2.88  | 5.01 | 1.03                              |
| GI-40    | 1.01 | 16.93 | .020 | .009 | .070 | 9.46 | 2.92  | 4.90 | 0.0                               |
| GI-42    | .78  | 25.69 | .014 | .014 | .085 | 9.73 | 3.46  | 5.13 | 0.16                              |
| GB-94    | 1.02 | 24.54 | .014 | .009 | .088 | 9.72 | 3.56  | 5.01 | 0.50                              |
| GI-43    | 1.00 | 26.09 | .014 | .016 | .028 | 9.73 | 5.00  | 5.00 | 1.2                               |
| GL-18    | .94  | 21.60 | .008 | .014 | .170 | 9.25 | 7.92  | 5.10 | 0.19                              |
| GL-19    | 1.00 | 22.18 | .010 | .016 | .052 | 9.32 | 11.68 | 5.06 | 1.65                              |

Nickel in controlled amounts is necessary along with the chromium to impart the desired oxidation resistance to the steel. Referring to FIG. 3, curve 16 is a graphic illustration of the oxidation test results on the steels having the nickel contents as listed in Table II. As illustrated, the nickel content must be not less than about 1% in order to maintain an oxidation rate of not more than 10 mg./cm.<sup>2</sup> when subjected to a 1093° C. (2000° F.) temperature with the best results being obtained where the nickel is maintained in the range of 3% to 8%.

Aluminum has proven to be critical in the steel of this invention as is illustrated by reference to the following Table III which lists steels having the aluminum varying from 4% to 12% with 0.75% to 1.02% carbon, 16.93% to 25.92% manganese, 2.0% to 11.7% nickel and 5% to 10% chromium and the oxidation rate for the steels as tested at 1093° C. (2000° F.) for a time in excess of 50 hours.

Table III

| Heat No. | C    | Mn    | P    | S    | Si   | Al    | Ni    | Cr    | Weight Gain, mg./cm. <sup>2</sup> |
|----------|------|-------|------|------|------|-------|-------|-------|-----------------------------------|
| GL-10    | 1.01 | 22.23 | .010 | .016 | .088 | 4.01  | 7.82  | 5.08  | 183.90                            |
| GL-9     | 1.00 | 22.35 | .013 | .008 | .100 | 4.12  | 2.92  | 5.04  | 162.99                            |
| GL-8     | .75  | 22.29 | .013 | .010 | .120 | 4.29  | 3.01  | 5.06  | 175.50                            |
| GL-13    | 1.01 | 23.62 | .008 | .012 | .066 | 4.17  | 3.26  | 9.94  | 119.90                            |
| GL-16    | .97  | 22.29 | .015 | .011 | .033 | 4.17  | 7.88  | 10.03 | 95.50                             |
| RV-648   | .98  | 20.33 | .008 | .012 | .080 | 7.10  | 2.91  | 5.04  | 116.15                            |
| RV-761   | .99  | 25.92 | .006 | .009 | .033 | 7.06  | 3.44  | 10.03 | 113.51                            |
| RV-760   | .99  | 24.60 | .006 | .009 | .045 | 8.74  | 3.49  | 9.99  | 2.21                              |
| GJ-38    | 1.02 | 19.58 | .030 | .009 | .100 | 9.00  | 2.88  | 5.01  | 1.03                              |
| RV-649   | .99  | 19.93 | .008 | .012 | .070 | 9.08  | 2.07  | 5.04  | 6.6                               |
| GL-18    | .94  | 21.60 | .008 | .014 | .170 | 9.25  | 7.92  | 5.10  | .19                               |
| GL-17    | .97  | 22.41 | .011 | .011 | .080 | 9.25  | 7.96  | 10.31 | 1.11                              |
| GL-19    | 1.00 | 22.18 | .010 | .016 | .062 | 9.32  | 11.68 | 5.06  | 1.65                              |
| GJ-40    | 1.01 | 16.93 | .020 | .009 | .070 | 9.46  | 2.92  | 4.90  | 0.0                               |
| GI-42    | .78  | 25.69 | .014 | .014 | .085 | 9.73  | 3.46  | 5.13  | .16                               |
| GB-94    | 1.02 | 24.54 | .014 | .009 | .088 | 9.72  | 3.56  | 5.01  | .50                               |
| RV-762   | .99  | 25.11 | .007 | .009 | .038 | 11.49 | 3.50  | 5.18  | .16                               |

Referring to FIG. 4, curve 18 is a graphic illustration of the oxidation test results reported in Table III as plotted against the aluminum content. Curve 18 demonstrates that aluminum is just as critical in the present steel as the chromium and nickel contents. Thus with only 4% aluminum, the oxidation rate is greater than 100 mg./cm.<sup>2</sup> even with the chromium at 10% and is greater than 150 mg./cm.<sup>2</sup> where the chromium is at 5%. In order to maintain the oxidation rate at not more than

10 mg./cm.<sup>2</sup> as tested at 1093° C. (2000° F.), it is necessary to maintain the aluminum content at not less than 8% and, for best results, preferably in the range of 9% to 12% with the nickel and chromium within the limits specified.

While the curves of FIGS. 2, 3 and 4 clearly demonstrate the effect of each of chromium, nickel and aluminum, respectively, on the oxidation resistance of the steel of this invention, it has been found that there is a definite relationship of the total of these elements within the ranges stated and particularly the preferred ranges to insure the optimum oxidation resistance. Thus for consistent and optimum oxidation resistance the elements must be present within the ranges given in an amount so that the sum of  $\text{Ni} + \text{Cr} + (4 \times \text{Al})$  must be equal to or greater than 43 in order to insure that the oxidation rate is not in excess of 10 mg./cm.<sup>2</sup> as tested at 1093° C. (2000° F.) for from 50 to 100 hours.

In order to demonstrate the necessity for the foregoing relationship, reference may be had to the following Table IV in which certain of the steels of the foregoing tables as well as additional steels are listed in an order dependent upon an increase in the value of  $\text{Ni} + \text{Cr} + (4 \times \text{Al})$ .

Table IV

| Heat No. | C    | Mn    | P    | S    | Si   | Al    | Ni    | Cr    | Weight Gain, mg./cm. <sup>2</sup> | [Ni+Cr+(4×Al)] |
|----------|------|-------|------|------|------|-------|-------|-------|-----------------------------------|----------------|
| FY-9     | .99  | 19.41 | .011 | .013 | .009 | 4.13  | 7.75  |       | 82.90                             | 24.27          |
| GL-9     | 1.00 | 22.35 | .013 | .008 | .100 | 4.12  | 2.92  | 5.04  | 162.99                            | 24.44          |
| GL-8     | .75  | 22.29 | .013 | .010 | .120 | 4.29  | 3.01  | 5.06  | 175.50                            | 25.23          |
| GL-10    | 1.01 | 22.23 | .010 | .016 | .038 | 4.01  | 7.82  | 5.08  | 183.90                            | 28.94          |
| GL-13    | 1.01 | 23.62 | .008 | .012 | .066 | 4.17  | 3.26  | 9.94  | 119.90                            | 29.88          |
| GL-16    | .97  | 22.29 | .015 | .011 | .033 | 4.17  | 7.88  | 10.03 | 95.50                             | 34.59          |
| RV-648   | .98  | 20.33 | .008 | .012 | .080 | 7.10  | 2.91  | 5.04  | 116.15                            | 36.35          |
| RV-650   | .99  | 20.16 | .003 | .011 | .066 | 8.60  | 0.50  | 5.00  | 13.00                             | 39.90          |
| FR-34    | .97  | 23.97 | .013 | .015 | .150 | 9.32  | 3.85  |       | 10.10                             | 41.13          |
| RV-761   | .99  | 25.92 | .006 | .009 | .033 | 7.06  | 3.44  | 10.03 | 113.51                            | 41.71          |
| GI-47    | 1.01 | 27.36 | .018 | .012 | .066 | 9.19  | 0.15  | 5.36  | 86.60                             | 42.27          |
| RV-649   | .99  | 19.93 | .008 | .012 | .070 | 9.08  | 2.07  | 5.04  | 6.60                              | 43.43          |
| GJ-38    | 1.02 | 19.58 | .030 | .009 | .100 | 9.00  | 2.88  | 5.01  | 1.03                              | 43.89          |
| GJ-40    | 1.01 | 16.93 | .020 | .009 | .070 | 9.48  | 2.92  | 4.90  | .00                               | 45.66          |
| RV-698   | 1.00 | 28.42 | .011 | .010 | .052 | 9.76  | 3.05  | 5.16  | 4.02                              | 47.25          |
| GB-94    | 1.02 | 24.54 | .014 | .009 | .038 | 9.72  | 3.56  | 5.01  | .60                               | 47.45          |
| GI-42    | .78  | 25.69 | .014 | .014 | .088 | 9.73  | 3.46  | 5.13  | .16                               | 47.51          |
| RV-788   | .95  | 24.94 | .003 | .009 | .042 | 9.50  | 0.99  | 8.98  | .40                               | 47.97          |
| RV-760   | .99  | 24.60 | .006 | .009 | .045 | 8.74  | 3.49  | 9.99  | .21                               | 48.44          |
| GI-43    | 1.00 | 26.09 | .014 | .016 | .028 | 9.73  | 5.00  | 5.00  | 1.20                              | 48.92          |
| GI-45    | 1.03 | 26.18 | .018 | .017 | .100 | 9.26  | 3.43  | 9.34  | .91                               | 49.81          |
| GI-44    | 1.03 | 26.15 | .017 | .014 | .047 | 9.80  | 3.42  | 7.25  | 1.10                              | 49.87          |
| GL-18    | .94  | 21.60 | .008 | .014 | .170 | 9.25  | 7.92  | 5.10  | .19                               | 50.02          |
| GL-19    | 1.00 | 22.18 | .010 | .016 | .052 | 9.32  | 11.68 | 5.06  | 1.65                              | 54.02          |
| RV-762   | .99  | 25.11 | .007 | .009 | .033 | 11.49 | 3.50  | 5.18  | .16                               | 54.64          |
| GL-17    | .97  | 22.41 | .011 | .011 | .080 | 9.25  | 7.96  | 10.31 | 1.11                              | 55.27          |

The foregoing relationship is demonstrated graphically in FIG. 5 in which the measured oxidation rates of the steels of Table IV are plotted against the sum of  $\text{Ni} + \text{Cr} + (4 \times \text{Al})$  and a parameter is drawn to show the definite band resulting. As is clearly evident from FIG. 5 only those steels having the elements within the ranges given hereinbefore and in which  $\text{Ni} + \text{Cr} + (4 \times \text{Al}) \geq 43$  will have the required low oxidation rate.

While reference has been made hereinbefore to the effect of nickel and chromium, it must be emphasized that the oxidation resistance of the steel cannot be improved simply by increasing the quantity of either or both of these elements. Instead the aluminum content is also critical and essential regardless of any such increase in the nickel and chromium contents. While this has been substantiated by the showing made in FIGS. 2 and 5, it becomes clearer when the results obtained on steels containing four different levels of aluminum are examined. For this purpose the steels identified hereinbefore in the specification and in Tables I, II, III and IV have been plotted in FIG. 6 which, while shown as a parallelogram is actually the lower left hand portion of a triaxial diagram in which chromium and nickel contents of the different steels are plotted against the balance of their compositions and for purpose of clarity the different heat numbers are identified on the parallelogram for a ready comparison. Any steel having an oxidation rate not in excess of 10 mg./cm.<sup>2</sup> is classified as good and those in excess of

such rate are classified as bad with the symbols representing different levels of aluminum as indicated.

Referring to the plots on FIG. 6, it becomes clear that the required oxidation rate is not obtained simply by increasing nickel and chromium but that instead the aluminum content is also critical. Thus as indicated GL-16 which has about 10% chromium and about 7.9% nickel but only about 4% aluminum has a poor oxidation rate of 95.5 mg./cm.<sup>2</sup>, whereas a comparable steel GL-17 having about 10% chromium and about 7.9% nickel but in which the aluminum is 9.25% has an excellent oxidation rate of 1.11 mg./cm.<sup>2</sup>. The same comparison may be made for the plots of GL-10 and GL-18, the main difference therebetween being that GL-10 having only about 4% aluminum has a poor oxidation rate and GL-18 having about 9.25% aluminum with the other elements being approximately the same as those for GL-10, has an excellent oxidation rate. This is also pictorially illustrated in a comparison of RV-761 and RV-760 as well as by the comparison of GL-8 and GL-9 with RV-698 and a comparison of RV-648 with GJ-38 and GJ-40. FIG. 6 clearly illustrates the necessity to maintain the elements within the critical limits previously described.

While it has been stated that the nickel may be present in an amount ranging from 1% to 12%, 3% is preferred as the lower limit in order to obtain fairly consistent oxidation resistance properties. On the other hand, while up to 12% nickel will impart excellent oxidation resistance properties, it is preferred to limit the nickel to not more than 8% since such element is relatively expensive as compared to iron. Further since nickel is an austenitizer and aluminum and chromium are ferritizers in iron-base steel alloys, it has been found that where more than about 8% nickel is utilized, that the nickel enters into a second magnetic phase along with the aluminum and chromium with the result that embrittlement and cracking is sometimes encountered during the processing of the resulting steel which contains in excess of 8% nickel. Since the aluminum and chromium, where present in the upper portion of the ranges given, cooperate to effect a duplex structure of austenite as well as the second magnetic phase with the nickel where the nickel is over 8%, that the combined chromium and aluminum contents should not exceed about 19.5% so as to prevent the formation of a brittle composition.

The steel of this invention may be annealed at temperatures of 1038° C. (1900° F.) to 1149° C. (2100° F.) and air cooled or water quenched therefrom to soften it to place it in a condition for forming into different shapes or for cold drawing into wire, the time of the anneal being dependent upon the mass to be so formed or drawn.

For example, a rod of the steel of Heat GB-94 when annealed for 30 minutes at 1093° C. (2000° F.) and water quenched had a  $R_c$  hardness of 29, a 0.2% yield strength of 99,400 pounds per square inch, a tensile strength of 133,700 pounds per square inch, a percent elongation in 1 inch of 51 and a reduction of area of 59%.

The steel of this invention has a high room temperature electrical resistivity of from 130 to 160 microhm-centimeters. For example, a typical steel as represented by the composition of Heat GB-94 has a room temperature resistivity of 156.8 microhm-centimeters as compared to the room temperature resistivity of 100 microhm-centimeters of the well known Alloy A referred to hereinbefore. Since the steel of this invention has a high resistivity, the steel is useful as the heating element in space heaters of all types including furnaces, ovens and stoves or heaters for home or other building heaters. In contrast to the well known Alloy A, since the steel of this invention has such a high resistivity a given heater element formed from a wire or ribbon of my steel can have a diameter or cross sectional area 50% larger than a similar heater element formed from Alloy A with a resulting increase in strength and surface area available for heat radiation. Such an increase in cross sectional and surface area makes it possible to operate the resulting heater in heat exchanger or power control applications at considerably lower temperatures than similar heaters formed of Alloy A for a given length of heater element and power or B.t.u. output. This characteristic found with the steel of the present invention is of extreme importance where maximum current levels and maximum temperatures must be considered in the design of the heaters.

It has also been found that the steel of this invention has a smaller coefficient of resistance change vs. temperature than that of conventional heater materials. For example, a representative steel of this invention Heat No. GK-20 having a density of 6.724 gm./cm.<sup>3</sup> and having an analysis of 0.97% carbon, 22.98% manganese, 0.020% phosphorus, 0.011% sulfur, 0.13% silicon, 9.24% aluminum, 3.26% nickel, 5.18% chromium and the balance iron when formed into a heater wire and tested had an electrical resistivity of 144.4 microhm-centimeters and a coefficient of resistance change over a temperature range of -80° C. (-112° F.) to +100° C. (+212° F.) as shown by curve 20 of FIG. 7. Such resistance change may be readily compared to that of the well known Alloy A as illustrated by curve 22 of FIG. 7. As will be seen there is substantially zero change in the coefficient of resistance of the steel of Heat No. GK-20 over the temperature range of -19° C. (-2.2° F.) to +20° C. (+68° F.) and that above such temperature any change therein is at a substantially constant and considerably lower rate than that of Alloy A. Likewise, it is seen that the steel of Heat No. GK-20 has a total change in coefficient of resistance of only about 0.13 ohm/ohm as measured over the wide range of -40° C. (-40° F.) to +45° C. (+113° F.). Such steel, having a low coefficient of resistance change up to 100° C. (212° F.), is readily formed into precise wire and tape resistors of all types and is useful as meter shunts as well as in high wattage, self-supporting or other cast grid, wire or tape resistors.

As is evident from curve 20 of FIG. 7, the steel represented by Heat GK-20 has a negative coefficient of resistance at temperatures below 0° C. (32° F.) which renders it particularly suitable for use in temperature compensating and temperature sensing devices. In addition since the steel has an austenitic structure it has been found that it is free from magnetostriction dimensional changes when subjected to alternating electric currents thereby rendering it suitable for applications where magnetostriction noise is objectionable.

As will be appreciated and as shown in the analysis of

the steels given in the foregoing tables the steel of this invention will usually contain small amounts of incidental impurities. Thus the alloys may contain up to 0.04% phosphorus, up to 0.03% sulfur and up to 0.50% silicon. Preferably phosphorus is maintained at less than 0.02% maximum, silicon at less than 0.20% maximum and sulfur at less than 0.015% maximum. However, in some instances where it is desired to improve machinability, the sulfur may be up to 0.5%. Usually phosphorus, sulfur and silicon will be present in a total amount of not more than 0.5%. In the composition ranges and analysis given hereinbefore, the percentages given in all instances are weight percentages.

I claim:

1. A low density, ductile, high strength, austenitic steel consisting essentially of, 0.50% to 1% carbon, 17% to 30% manganese, 8% to 12% aluminum, 1% to 12% nickel, 3% to 11% chromium, and the balance iron with incidental impurities, the combined chromium and aluminum contents of said steel being less than about 19.5% when the nickel content is more than about 8%, said steel being characterized by high oxidation resistance at temperatures in excess of 871° C. (1600° F.), high electrical resistivity, low coefficient of electrical resistance change vs. temperature and being substantially free from magnetostriction change in dimension when subjected to alternating electrical currents.

2. A low density, ductile, high strength, austenitic steel consisting essentially of 0.75% to 1% carbon, 17% to 30% manganese, 9% to 12% aluminum, 3% to 8% nickel, 5% to 10% chromium, and the balance iron with incidental impurities, said steel being characterized by high oxidation resistance at temperatures in excess of 871° C. (1600° F.), high electrical resistivity, low coefficient of electrical resistance change vs. temperature and being substantially free from magnetostriction change in dimension when subjected to alternating electrical currents.

3. A low density, ductile, high strength, austenitic steel consisting of, 0.50% to 1% carbon, 17% to 30% manganese, 8% to 12% aluminum, 1% to 12% nickel, and 3% to 11% chromium, 0.04% maximum phosphorus, 0.03% maximum sulfur, 0.2% maximum silicon, and the balance iron, the combined chromium and aluminum contents of said steel being less than about 19.5% when the nickel content is more than about 8%, said steel being characterized by high oxidation resistance at temperatures in excess of 871° C. (1600° F.), high electrical resistivity, low coefficient of electrical resistance change vs. temperature and being substantially free from magnetostriction change in dimension when subjected to alternating electrical currents.

4. A low density, ductile, high strength, austenitic steel consisting of, 0.75% to 1% carbon, 17% to 30% manganese, 9% to 12% aluminum, 3% to 8% nickel, 5% to 10% chromium, 0.02% maximum phosphorus, 0.015% maximum sulfur, 0.2% maximum silicon, and the balance iron, said steel being characterized by high oxidation resistance at temperatures in excess of 871° C. (1600° F.), high electrical resistivity, low coefficient of electrical resistance change vs. temperature and being substantially free from magnetostriction change in dimension when subjected to alternating electrical currents.

5. A low density, ductile, high strength, austenitic steel consisting essentially of, 0.50% to 1% carbon, 17% to 30% manganese, 8% to 12% aluminum, 1% to 12% nickel, 3% to 11% chromium, and the balance iron with incidental impurities, the combined chromium and aluminum contents of said steel being less than about 19.5% when the nickel content is more than about 8% and the sum of the nickel and chromium contents plus four times the aluminum content is not less than 43, said steel being characterized by high oxidation resistance at temperatures in excess of 871° C. (1600° F.), high electrical resistivity, low coefficient of electrical resistance change vs.

temperature and being substantially free from magnetostriction change in dimension when subjected to alternating electrical currents.

6. A low density, ductile, high strength, austenitic steel consisting essentially of, 0.75% to 1% carbon, 17% to 30% manganese, 9% to 12% aluminum, 3% to 8% nickel, 5% to 10% chromium, and the balance iron with incidental impurities, the sum of the percentages of the chromium content and nickel content plus four times the aluminum content being not less than 43, said steel being characterized by high oxidation resistance at temperatures in excess of 871° C. (1600° F.), high electrical resistivity, low coefficient of electrical resistance change vs. temperature and being substantially free from magnetostriction change in dimension when subjected to alternating electrical currents.

7. A heating element formed of an austenitic steel having an electrical resistivity of from 130 to 160 microhm-centimeters and high oxidation resistance, said steel having a composition analysis consisting essentially of 0.50% to 1% carbon, 17% to 30% manganese, 8% to 12% aluminum, 1% to 12% nickel, 3% to 11% chromium, and the balance iron with incidental impurities, the combined chromium and aluminum contents of said steel being less than about 19.5% when the nickel content is more than about 8%.

8. A heating element formed of an austenitic steel having an electrical resistivity of from 130 to 160 microhm-centimeters and high oxidation resistance, said steel hav-

ing an analysis consisting essentially of from 0.75% to 1% carbon, 17% to 30% manganese, 9% to 12% aluminum, 3% to 8% nickel, 5% to 10% chromium and the balance iron with incidental impurities.

5. 9. A low density, ductile, high strength, austenitic steel consisting of, about 1.0% carbon, about 24.5% manganese, about 9.70% aluminum, 3.5% nickel, 5.0% chromium, and the balance iron with incidental impurities.

10. A low density, ductile, high strength, austenitic steel consisting of, 0.50% to 1% carbon, 17% to 30% manganese, 8% to 12% aluminum, 1% to 12% nickel, 3% to 11% chromium, up to 0.5% sulfur, and the balance iron with incidental impurities, and in which the sum of the nickel and chromium contents plus four times the aluminum content is not less than 43.

11. An electrical resistor heating element formed of an austenitic steel having a composition consisting essentially of, 0.50% to 1% carbon, 17% to 30% manganese, 8% to 12% aluminum, 1% to 12% nickel, 3% to 11% chromium, and the balance iron with not more than 0.5% incidental impurities, and in which the sum of the nickel and chromium contents plus four times the aluminum content is not less than 43, and in which the combined chromium and aluminum contents are less than about 19.5% when the nickel content is more than about 8%, said heating element being characterized by having an electrical resistivity of from 130 to 160 microhm-centimeters.

No references cited.